

## UNITED STATES PATENT OFFICE

GEORGE R. LOCKHART, OF PROVIDENCE, RHODE ISLAND, ASSIGNOR TO MANVILLE JENCKES COMPANY, OF PAWTUCKET, RHODE ISLAND, A CORPORATION OF RHODE ISLAND

## MANUFACTURE OF RAYON

No Drawing.

Application filed November 9, 1928. Serial No. 318,308.

The invention relates to the manufacture of rayon (artificial silk) and more particularly to the production of dyed rayon thread formed under the viscose process.

5 The present invention has for its object to produce from a viscose solution lustrous thread of high tensile strength which is dyed to its final color upon being precipitated in the setting bath.

10 In the manufacture of rayon or artificial silk from a viscose solution as usually carried out, the viscose is precipitated in the form of slender filaments by forcing the viscose solution through a spinneret into a precipitating or setting bath. The filaments are then gathered together to form a thread and the thread is either wound on a bobbin or guided to a centrifuge pot by which it is twisted and formed into a so-called "cake".

15 From the bobbin or "cake" as the case may be, the thread is wound on reels to form skeins which are then subjected to a series of operations to prepare the rayon for commercial use. These operations include washing, stretching, drying, desulphurizing, 20 bleaching, dyeing, etc. The rayon is then finally spooled and is ready for commercial use.

25 The results produced by the usual methods of dyeing rayon thread in skein form, however, are not entirely satisfactory. Not only is the operation expensive on account of the high cost of labor, materials, and apparatus, but what is of more importance, the cellulose 30 of which the thread is composed does not dye readily or uniformly in all cases, variations in color being produced for various reasons, as for instance, where portions of the thread have been converted from hydrocellulose 35 into oxy cellulose during the drying operation, or where the thread is not of uniform thickness, or where all portions of the skein have not been subjected to the same amount 40 of dyeing fluid. Moreover, on account of the variations in the affinity for the dyestuffs of different lots of rayon thread, it has been found extremely difficult to produce exactly 45 the desired color for any given lot of rayon, and practically impossible to match a color,

which has been once produced, with any degree of accuracy.

It is the object of the present invention to provide a method for dyeing rayon made from viscose which will avoid these objections and provide a uniformly dyed thread the color of which may be determined with mathematical accuracy.

55 With this object in view, the applicant proposes to insert the dyestuff in the viscose solution so that when the viscose is forced through the spinnerets into the coagulating bath, viscose filaments will be produced having the desired color and requiring no further treatment so far as the dyeing operation 60 is concerned. So far as the applicant is aware, no one up to the present time has successfully dyed rayon made from viscose in the viscose solution, so that the filaments produced from the setting bath are in their final 65 dyed state. Applicant's experiments, for instance, have indicated that it is impracticable to put direct dyes or pigments into the viscose solution, inasmuch as these substances tend either to materially weaken the thread 70 produced or make the viscose entirely unsuitable to be drawn out into filaments through the spinnerets. Similarly, where the applicant has attempted to use indanthrene or sulphur dyes, mixing them in the 75 usual manner with a reducing agent to render them soluble, and then adding them to the viscose solution, the tendency has been to stabilize the viscose solution and prevent proper aging and obtaining the right viscosity for spinning the viscose.

80 In carrying out the present method for successfully dyeing in the viscose solution, the applicant employs dyes which must be put into a state of reduction to render them 85 soluble, of which examples are indanthrene and sulphur colors, and these dyes are put and held in a reduced state by the viscose solution until after the viscose has been forced through the spinnerets into the setting bath, 90 and are then fixed in the newly formed viscose filaments to produce the required color. For reducing and holding the dye in a reduced state, the chemicals are utilized which 95 are formed in the process of viscose manufac- 100

ture. In the course of the usual process of manufacture of rayon from a viscose solution, the cellulose zanthate is dissolved in a 3% caustic solution. It is at this point that the dye for coloring the cellulose is added. In order to dissolve a given amount of the zanthate, a definite amount of 3% caustic solution is required as will be readily understood by those skilled in the art. Some of this 3% caustic solution is taken and mixed with the dye to make it into a paste and the remainder of the caustic solution is added to the zanthate. The dye in paste form is then added to the viscose in the dissolving machine. By the usual mechanical methods of stirring, the viscose becomes thoroughly dissolved while at the same time the dyestuff is well mixed in the solution. The viscose solution serves as a reducing agent for the dye and holds it permanently in a reduced state during the subsequent aging and until it reaches the setting bath.

The setting bath may be that usually employed in the viscose process of producing rayon, i. e., sulphuric acid and sodium sulphate, and acts as an oxidizing agent for the dyestuff as the filaments are formed in the bath.

At the same time that the viscose is drawn from the spinnerets into filaments in the setting bath, the dyestuff in the precipitated viscose becomes oxidized and is fixed in the substance of the filaments to give the thread its final color. Due to the method here employed of mixing the dyestuff thoroughly into the viscose solution and holding it in a reduced state until the viscose is precipitated in the setting bath, an even distribution of the coloring matter is secured, as filaments are produced, to insure a constant shade in the finished thread. The dyestuff, being in a reduced state and in solution, is a constituent of that part of the viscose solution which is precipitated out in the setting bath to form filaments. The association of the dyestuff with the cellulose compounds of the viscose solution is so intimate, that possibly the molecules themselves are affected. Whether the association results in a chemical change or is merely mechanical, the dyestuff is uniformly distributed throughout the filaments and as the dyestuff becomes oxidized, the filaments are thoroughly impregnated with the desired color without regard to their size. Also, inasmuch as the color has been finally fixed in the filament, any subsequent change of the fiber from hydrocellulose to oxycellulose will not result in any change in the color which has been originally produced.

A further advantage of the method herein disclosed of producing dyed rayon thread rests in the fact that all of the dyestuff put into the solution is apparently taken up by the viscose. Consequently there is no waste of the dyestuff such as is found in the usual

methods of handling vat dyes where the skeins or hanks of rayon when submerged in a dye bath take up only a portion of the dye in the solution. Furthermore, since it is known that all of the dyestuff will be taken up by the precipitated viscose in even proportion, it is possible by measuring the dyestuff and other ingredients used in making the viscose solution, to determine with mathematical accuracy in advance the shade of color which will be produced.

The nature and objects of the invention having been indicated and the preferred manner of carrying out the invention having been specifically described, what is claimed is:—

1. The process of producing dyed rayon thread which comprises precipitating cellulose in filament form from a viscose solution while impregnated with dyestuff in a reduced state, and oxidizing the dyestuff to fix the color in the filaments.

2. The process of producing dyed rayon thread which comprises inserting in the viscose solution a dyestuff which may be reduced in an alkaline solution to render it soluble, utilizing the chemical compounds present in the viscose to reduce the dyestuff and hold it in solution, precipitating filaments from the viscose solution in a setting bath, and utilizing the setting bath to oxidize the dyestuff in the filaments to produce filaments of the required color.

3. The process of producing dyed rayon thread which comprises inserting in the viscose solution a dyestuff which may be reduced in an alkaline solution to render it soluble, utilizing the chemical compounds present in the viscose to reduce the dyestuff and hold it in solution, precipitating filaments from the viscose solution in a setting bath, and oxidizing the dyestuff in the filaments to produce filaments of the required color.

4. The process of producing rayon thread which comprises inserting an indanthrene dyestuff in the viscose solution, holding the dyestuff in a reduced state in the solution, precipitating filaments from the viscose in a setting bath, and oxidizing the dyestuff to fix the color in the filaments.

5. The process of producing dyed rayon thread which comprises adding a dyestuff which may be reduced in an alkaline solution to render it soluble to cellulose zanthate and a three percent caustic solution, thoroughly mixing the dyestuff with the solution to reduce the dyestuff and hold it in a reduced state, precipitating cellulose in the form of filaments from the viscose solution in a setting bath, and oxidizing the dyestuff to fix the color in the filaments.

6. The process of producing rayon thread which comprises inserting a dye of the group consisting of sulphur dyes and indanthrene

or vat dyes in the viscose solution, holding the dyestuff in a reduced state in the solution, precipitating filaments from the viscose in a setting bath, and oxidizing the dyestuff to fix the color in the filaments.

5 In testimony whereof I have signed my name to this specification.

GEORGE R. LOCKHART.

10

15

20

25

30

35

40

45

50

55

60